



US008894738B2

(12) **United States Patent**  
**Jacobsen et al.**

(10) **Patent No.:** **US 8,894,738 B2**  
(45) **Date of Patent:** **Nov. 25, 2014**

(54) **TITANIUM ALLOY**

(75) Inventors: **Lance E. Jacobsen**, Minooka, IL (US);  
**Adam John Benish**, Crest Hill, IL (US)

(73) Assignee: **Cristal Metals Inc.**, Hunt Valley, MD  
(US)

(\*) Notice: Subject to any disclaimer, the term of this  
patent is extended or adjusted under 35  
U.S.C. 154(b) by 158 days.

(21) Appl. No.: **12/879,598**

(22) Filed: **Sep. 10, 2010**

(65) **Prior Publication Data**

US 2010/0329919 A1 Dec. 30, 2010

(56)

**References Cited**

U.S. PATENT DOCUMENTS

|           |   |         |                 |
|-----------|---|---------|-----------------|
| 1,771,928 | A | 7/1930  | Jung            |
| 2,205,854 | A | 6/1940  | Kroll           |
| 2,607,675 | A | 8/1952  | Gross           |
| 2,647,826 | A | 8/1953  | Jordan          |
| 2,816,828 | A | 12/1957 | Benedict et al. |
| 2,823,991 | A | 2/1958  | Kamlet          |
| 2,827,371 | A | 3/1958  | Quin            |
| 2,835,567 | A | 5/1958  | Willcox         |
| 2,846,303 | A | 8/1958  | Keller et al.   |
| 2,846,304 | A | 8/1958  | Keller et al.   |

(Continued)

FOREIGN PATENT DOCUMENTS

|    |               |        |
|----|---------------|--------|
| AU | 2003263081    | 6/2004 |
| WO | WO96/04407    | 2/1996 |
| WO | WO2005/019485 | 3/2005 |
| WO | WO2005/021807 | 3/2005 |

OTHER PUBLICATIONS

Peter et al, Structure and properties of titanium and titanium alloys,  
book edited by Leyens et al, Titanium and titanium alloys, Wiley-VCHGmbH&Co. KGaA, copyright 2003, pp. 1-23.\*

(Continued)

Primary Examiner — Jie Yang

(74) Attorney, Agent, or Firm — Dunlap Codding, P.C.

(57) **ABSTRACT**

A titanium base alloy powder having lesser amounts of aluminum and vanadium with an alkali or alkaline earth metal being present in an amount of less than about 200 ppm. The alloy powder is neither spherical nor angular and flake shaped. 6/4 alloy is specifically disclosed having a packing fraction or tap density between 4 and 11%, as is a method for making the various alloys.

35 Claims, 12 Drawing Sheets



| (56)                  | References Cited  |                                        |
|-----------------------|-------------------|----------------------------------------|
| U.S. PATENT DOCUMENTS |                   |                                        |
| 2,882,143 A           | 4/1959            | Schmidt                                |
| 2,882,144 A           | 4/1959            | Follows et al.                         |
| 2,890,112 A           | 6/1959            | Winter                                 |
| 2,895,823 A           | 7/1959            | Lynskey                                |
| 2,915,382 A           | 12/1959           | Hellier et al.                         |
| 2,941,867 A           | 6/1960            | Maurer                                 |
| 2,944,888 A           | 7/1960            | Quin                                   |
| 3,058,820 A           | 10/1962           | Whitehurst                             |
| 3,067,025 A           | 12/1962           | Chisholm                               |
| 3,085,871 A           | 4/1963            | Griffiths                              |
| 3,085,872 A           | 4/1963            | Kenneth                                |
| 3,113,017 A           | 12/1963           | Homme                                  |
| 3,331,666 A           | 7/1967            | Robinson et al.                        |
| 3,519,258 A           | 7/1970            | Ishizuka                               |
| 3,535,109 A           | 10/1970           | Ingersoll                              |
| 3,650,681 A           | 3/1972            | Sugahara et al.                        |
| 3,825,415 A           | 7/1974            | Johnston et al.                        |
| 3,836,302 A           | 9/1974            | Kaukeinen                              |
| 3,847,596 A           | 11/1974           | Holland et al.                         |
| 3,867,515 A           | 2/1975            | Bohl et al.                            |
| 3,919,087 A           | 11/1975           | Brumagim                               |
| 3,927,993 A           | 12/1975           | Griffin                                |
| 3,943,751 A           | 3/1976            | Akiyama et al.                         |
| 3,966,460 A           | 6/1976            | Spink                                  |
| 4,007,055 A           | 2/1977            | Whittingham                            |
| 4,009,007 A           | 2/1977            | Fry                                    |
| 4,017,302 A           | 4/1977            | Bates et al.                           |
| 4,070,252 A           | 1/1978            | Bonsack                                |
| 4,128,421 A           | 12/1978           | Marsh et al.                           |
| 4,141,719 A           | 2/1979            | Hakko                                  |
| 4,149,876 A           | 4/1979            | Rerat                                  |
| 4,190,442 A           | 2/1980            | Patel                                  |
| 4,331,477 A           | 5/1982            | Kubo et al.                            |
| 4,373,947 A *         | 2/1983            | Buttner et al. .... 75/228             |
| 4,379,718 A           | 4/1983            | Grantham et al.                        |
| 4,401,467 A           | 8/1983            | Jordan                                 |
| 4,402,741 A           | 9/1983            | Pollet et al.                          |
| 4,414,188 A           | 11/1983           | Becker                                 |
| 4,423,004 A           | 12/1983           | Ross                                   |
| 4,425,217 A           | 1/1984            | Beer                                   |
| 4,432,813 A           | 2/1984            | Williams                               |
| 4,445,931 A           | 5/1984            | Worthington                            |
| 4,454,169 A           | 6/1984            | Hinden et al.                          |
| 4,518,426 A           | 5/1985            | Murphy                                 |
| 4,519,837 A           | 5/1985            | Down                                   |
| 4,521,281 A           | 6/1985            | Kadija                                 |
| 4,555,268 A           | 11/1985           | Getz                                   |
| 4,556,420 A           | 12/1985           | Evans et al.                           |
| 4,604,368 A           | 8/1986            | Reeve                                  |
| 4,606,902 A           | 8/1986            | Ritter                                 |
| RE32,260 E            | 10/1986           | Fry                                    |
| 4,687,632 A           | 8/1987            | Hurd                                   |
| 4,689,129 A           | 8/1987            | Knudsen                                |
| 4,725,312 A           | 2/1988            | Seon et al.                            |
| 4,828,008 A           | 5/1989            | White et al.                           |
| 4,830,665 A           | 5/1989            | Winand                                 |
| 4,839,120 A           | 6/1989            | Baba et al.                            |
| 4,877,445 A           | 10/1989           | Okudaira et al.                        |
| 4,897,116 A           | 1/1990            | Scheel                                 |
| 4,902,341 A           | 2/1990            | Okudaira et al.                        |
| 4,915,729 A           | 4/1990            | Boswell et al.                         |
| 4,923,577 A           | 5/1990            | McLaughlin et al.                      |
| 4,940,490 A           | 7/1990            | Fife et al.                            |
| 4,941,646 A           | 7/1990            | Stelts et al.                          |
| 4,985,069 A           | 1/1991            | Traut                                  |
| 5,028,491 A           | 7/1991            | Huang et al.                           |
| 5,032,176 A           | 7/1991            | Kametani et al.                        |
| 5,055,280 A           | 10/1991           | Nakatani et al.                        |
| 5,064,463 A           | 11/1991           | Ciomek                                 |
| 5,082,491 A           | 1/1992            | Rerat                                  |
| 5,147,451 A           | 9/1992            | Leland                                 |
| 5,149,497 A           | 9/1992            | McKee et al.                           |
| 5,160,428 A           | 11/1992           | Kuri                                   |
| 5,164,346 A           | 11/1992           | Giunchi et al.                         |
| 5,167,271 A           | 12/1992           | Lange et al.                           |
|                       |                   | 5,176,741 A 1/1993 Bartlett et al.     |
|                       |                   | 5,176,810 A 1/1993 Volotinen et al.    |
|                       |                   | 5,211,741 A 5/1993 Fife                |
|                       |                   | 5,259,862 A 11/1993 White et al.       |
|                       |                   | 5,338,379 A 8/1994 Kelly               |
|                       |                   | 5,356,120 A 10/1994 König et al.       |
|                       |                   | 5,427,602 A 6/1995 DeYoung et al.      |
|                       |                   | 5,437,854 A 8/1995 Walker et al.       |
|                       |                   | 5,439,750 A 8/1995 Ravenhall et al.    |
|                       |                   | 5,448,447 A 9/1995 Chang               |
|                       |                   | 5,460,642 A 10/1995 Leland             |
|                       |                   | 5,498,446 A 3/1996 Axelbaum et al.     |
|                       |                   | 5,580,516 A 12/1996 Kumar              |
|                       |                   | H1642 H 4/1997 Jenkins                 |
|                       |                   | 5,637,816 A 6/1997 Schneibel           |
|                       |                   | 5,779,761 A 7/1998 Armstrong et al.    |
|                       |                   | 5,897,830 A 4/1999 Abkowitz et al.     |
|                       |                   | 5,914,440 A 6/1999 Celik et al.        |
|                       |                   | 5,948,495 A 9/1999 Stanish et al.      |
|                       |                   | 5,951,822 A 9/1999 Knapick et al.      |
|                       |                   | 5,954,856 A 9/1999 Pathare et al.      |
|                       |                   | 5,958,106 A 9/1999 Armstrong et al.    |
|                       |                   | 5,986,877 A 11/1999 Pathare et al.     |
|                       |                   | 5,993,512 A 11/1999 Pargeter et al.    |
|                       |                   | 6,010,661 A 1/2000 Abe et al.          |
|                       |                   | 6,027,585 A 2/2000 Patterson et al.    |
|                       |                   | 6,040,975 A 3/2000 Mimura              |
|                       |                   | 6,099,664 A 8/2000 Davies              |
|                       |                   | 6,103,651 A 8/2000 Leitzel             |
|                       |                   | 6,136,062 A 10/2000 Loffelholz et al.  |
|                       |                   | 6,180,258 B1 1/2001 Klier              |
|                       |                   | 6,193,779 B1 2/2001 Reichert et al.    |
|                       |                   | 6,210,461 B1 4/2001 Elliott            |
|                       |                   | 6,238,456 B1 5/2001 Wolf et al.        |
|                       |                   | 6,309,570 B1 10/2001 Fellabaum         |
|                       |                   | 6,309,595 B1 10/2001 Rosenberg et al.  |
|                       |                   | 6,409,797 B2 6/2002 Armstrong et al.   |
|                       |                   | 6,432,161 B1 8/2002 Oda et al.         |
|                       |                   | 6,488,073 B1 12/2002 Blenkinsop et al. |
|                       |                   | 6,502,623 B1 1/2003 Schmitt            |
|                       |                   | 6,602,482 B2 8/2003 Kohler et al.      |
|                       |                   | 6,689,187 B2 2/2004 Oda                |
|                       |                   | 6,727,005 B2 4/2004 Gimondo et al.     |
|                       |                   | 6,745,930 B2 6/2004 Schmitt            |
|                       |                   | 6,824,585 B2 11/2004 Joseph et al.     |
|                       |                   | 6,861,038 B2 3/2005 Armstrong et al.   |
|                       |                   | 6,884,522 B2 4/2005 Adams et al.       |
|                       |                   | 6,902,601 B2 6/2005 Nie et al.         |
|                       |                   | 6,921,510 B2 7/2005 Ott et al.         |
|                       |                   | 6,955,703 B2 10/2005 Zhou et al.       |
|                       |                   | 7,041,150 B2 5/2006 Armstrong et al.   |
|                       |                   | 7,351,272 B2 4/2008 Armstrong et al.   |
|                       |                   | 7,410,610 B2 8/2008 Woodfield et al.   |
|                       |                   | 7,435,282 B2 10/2008 Armstrong et al.  |
|                       |                   | 7,445,658 B2 11/2008 Armstrong et al.  |
|                       |                   | 7,501,007 B2 3/2009 Anderson et al.    |
|                       |                   | 7,501,089 B2 3/2009 Armstrong et al.   |
|                       | 2002/005090 A1    | 1/2002 Armstrong et al.                |
|                       | 2002/0050185 A1   | 5/2002 Oda                             |
|                       | 2002/0152844 A1   | 10/2002 Armstrong et al.               |
|                       | 2002/0194953 A1 * | 12/2002 Rosenberg et al. .... 75/10.18 |
|                       | 2003/0061907 A1   | 4/2003 Armstrong et al.                |
|                       | 2003/0145682 A1   | 8/2003 Anderson et al.                 |
|                       | 2004/0123700 A1   | 7/2004 Zhou et al.                     |
|                       | 2005/0081682 A1   | 4/2005 Armstrong et al.                |
|                       | 2005/0150576 A1   | 7/2005 Venigalla                       |
|                       | 2005/0225014 A1   | 10/2005 Armstrong et al.               |
|                       | 2005/0284824 A1   | 12/2005 Anderson et al.                |
|                       | 2006/0086435 A1   | 4/2006 Anderson et al.                 |
|                       | 2006/0102255 A1   | 5/2006 Woodfield et al.                |
|                       | 2006/0107790 A1   | 5/2006 Anderson et al.                 |
|                       | 2006/0123950 A1   | 6/2006 Anderson et al.                 |
|                       | 2006/0150769 A1   | 7/2006 Armstrong et al.                |
|                       | 2006/0230878 A1   | 10/2006 Anderson et al.                |
|                       | 2007/0017319 A1   | 1/2007 Jacobsen et al.                 |
|                       | 2007/0079908 A1   | 4/2007 Jacobsen et al.                 |
|                       | 2007/0180951 A1   | 8/2007 Armstrong et al.                |
|                       | 2007/0180952 A1   | 8/2007 Lanin et al.                    |
|                       | 2008/0031766 A1   | 2/2008 Kogut et al.                    |

(56)

**References Cited**

U.S. PATENT DOCUMENTS

- 2008/0152533 A1 6/2008 Ernst et al.  
2008/0187455 A1 8/2008 Armstrong et al.  
2008/0199348 A1 8/2008 Armstrong et al.

OTHER PUBLICATIONS

- Kelto et al. "Titanium Powder Metallurgy—A Perspective"; Conference: Powder Metallurgy of Titanium Alloys, Las Vegas, Nevada, Feb. 1980, pp. 1-19.  
Mahajan et al. "Microstructure Property Correlation in Cold Pressed and Sintered Elemental Ti-6Al-4V Powder Compacts"; Conference:

Powder Metallurgy of Titanium Alloys, Las Vegas, Nevada, Feb. 1980, pp. 189-202.

Moxson et al. "Production and Applications of Low Cost Titanium Powder Products"; The International Journal of Powder Metallurgy, vol. 34, No. 5, 1998, pp. 45-47.

Gerdemann et al. "Characterization of a Titanium Powder Produced Through a Novel Continuous Process"; Published by Metal Powder Industries Federation, 2000, pp. 12.41-12.52.

Moxson et al. "Innovations in Titanium Powder Processing"; Titanium Overview, JOM, May 2000, p. 24.

\* cited by examiner



**FIGURE 1**



FIGURE 2



FIGURE 3



**FIGURE 4**



**FIGURE 5**



**FIGURE 6**



**FIGURE 7**



**FIGURE 8**



**FIGURE 9**



**FIGURE 10**



**FIGURE 11**



**FIGURE 12**

# 1

## TITANIUM ALLOY

### CROSS REFERENCE TO RELATED APPLICATIONS

The present application is a continuation of U.S. Ser. No. 11/186,724 filed Jul. 21, 2005 now abandoned.

### FIELD OF THE INVENTION

This invention relates to alloys of titanium having at least 50% titanium and most specifically to an alloy of titanium particularly useful in the aerospace and defense industries known as 6/4 which is about 6% by weight aluminum and about 4% by weight vanadium with the balance titanium and trace materials as made by the Armstrong process.

### BACKGROUND OF THE INVENTION

The ASTM B265 grade 5 chemical specifications for 6/4 require that vanadium is present in the amount of 4% $\pm$ 1% by weight and aluminum is present in the range of from about 5.5% to about 6.75% by weight. The alloy of the invention is produced by the Armstrong Process as previously disclosed in U.S. Pat. Nos. 5,779,761; 5,958,106 and 6,409,797, the entire disclosures of which are herein incorporated by reference. The aforementioned patents teach the Armstrong Process as it

as a reducing metal, it should be understood that various halides other than chlorine can be used and various reductants other than sodium can be used and the invention is broad enough to include those materials.

5 However, because the Armstrong Process over the past eleven years has been developed using molten sodium and chlorides, it is these materials which are referenced herein. During the production of titanium by the Armstrong Process, as disclosed in the previous patents, the steady state temperature of the reaction can be controlled by the amount of reductant metal and the amount of chloride being introduced. Although it is feasible to control the reaction temperature by varying the chloride concentration while keeping the amount of molten metal constant, the preferred method is to control the temperature of the reactant products by varying the amount of excess (over stoichiometric) reductant metal introduced into the reaction chamber. Preferably, the reaction is maintained at a steady state temperature of about 400° C. and at this temperature, as previously disclosed, the reaction can be maintained for very long periods of time without damage to the equipment while producing a relatively uniform product.

10 Heretofore, commercially pure (CP) titanium ASTM B265 grades 1, 2, 3 and 4 have been produced in over two hundred runs using the Armstrong Process and although a wide variety of operating parameters have been tested, certain results are inherent in the process. The ASTM B 265 spec sheet follows:

TABLE 1

| Element                                   | Chemical Requirements  |           |           |           |             |            |              |            |              |            |
|-------------------------------------------|------------------------|-----------|-----------|-----------|-------------|------------|--------------|------------|--------------|------------|
|                                           | Composition %<br>Grade |           |           |           |             |            |              |            |              |            |
| Element                                   | 1                      | 2         | 3         | 4         | 5           | 6          | 7            | 8          | 9            | 10         |
| Nitrogen max                              | 0.03                   | 0.03      | 0.05      | 0.05      | 0.05        | 0.05       | 0.03         | 0.02       | 0.03         | 0.03       |
| Carbon max                                | 0.10                   | 0.10      | 0.10      | 0.10      | 0.10        | 0.10       | 0.10         | 0.10       | 0.10         | 0.08       |
| Hydrogen <sup>B</sup> max                 | 0.015                  | 0.015     | 0.015     | 0.015     | 0.015       | 0.020      | 0.015        | 0.015      | 0.015        | 0.015      |
| Iron Max                                  | 0.20                   | 0.30      | 0.30      | 0.50      | 0.40        | 0.50       | 0.30         | 0.25       | 0.20         | 0.30       |
| Oxygen max                                | 0.18                   | 0.25      | 0.35      | 0.40      | 0.20        | 0.20       | 0.25         | 0.15       | 0.18         | 0.25       |
| Aluminum                                  | —                      | —         | —         | —         | 5.5 to 6.75 | 4.0 to 6.0 | —            | 2.5 to 3.5 | —            | —          |
| Vanadium                                  | —                      | —         | —         | —         | 3.5 to 4.5  | —          | —            | —          | 2.0 to 3.0   | —          |
| Tin                                       | —                      | —         | —         | —         | —           | 2.0 to 3.0 | —            | —          | —            | —          |
| Palladium                                 | —                      | —         | —         | —         | —           | —          | 0.12 to 0.25 | —          | 0.12 to 0.25 | —          |
| Molybdenum                                | —                      | —         | —         | —         | —           | —          | —            | —          | —            | 0.2 to 0.4 |
| Zirconium                                 | —                      | —         | —         | —         | —           | —          | —            | —          | —            | —          |
| Nickel                                    | —                      | —         | —         | —         | —           | —          | —            | —          | —            | 0.6 to 0.9 |
| Residuals <sup>C,D,E</sup><br>(each), max | 0.1                    | 0.1       | 0.1       | 0.1       | 0.1         | 0.1        | 0.1          | 0.1        | 0.1          | 0.1        |
| Residuals <sup>C,D,E</sup><br>(total) max | 0.4                    | 0.4       | 0.4       | 0.4       | 0.4         | 0.4        | 0.4          | 0.4        | 0.4          | 0.4        |
| Titanium <sup>F</sup>                     | remainder              | remainder | remainder | remainder | remainder   | remainder  | remainder    | remainder  | remainder    | remainder  |

<sup>A</sup>Analysis shall be completed for all elements listed in this Table for each grade. The analysis results for the elements not quantified in the Table need not be reported unless the concentration level is greater than 0.1% each or 0.4% total.

<sup>B</sup>Lower hydrogen may be obtained by negotiation with the manufacturer.

<sup>C</sup>Need not be reported.

<sup>D</sup>A residual is an element present in a metal or an alloy in small quantities inherent to the manufacturing process but not added intentionally.

<sup>E</sup>The purchaser may, in his written purchase order, request analysis for specific residual elements not listed in this specification. The maximum allowable concentration for residual elements shall be 0.1% each and 0.4% maximum total.

<sup>F</sup>The percentage of titanium is determined by difference.

relates to the production of various materials including alloys. The Armstrong Process includes the subsurface reduction of halides by a molten metal alkali or alkaline earth element or alloy. The development of the Armstrong Process has occurred from 1994 through the present, particularly as it relates to the production of titanium and its alloys using titanium tetrachloride as a source of titanium and using sodium as the reducing agent. Although this invention is described particularly with respect to titanium tetrachloride, aluminum trichloride and vanadium tetrachloride and sodium

60 Production of titanium powder by the Armstrong Process inherently produces powder in which the average diameter of individual particle is less than a micron. During distillation at 500 to 600° C., the particles agglomerate and have an average agglomerated particle diameter in the range of from about 3.3 to about 1.3 microns. Particle diameters are based on a calculated size of a sphere from a surface area, such as BET. For 65 agglomerated particles, the calculated average diameters were based on surface area measurements in a range of from about 0.4 to about 1.0 m<sup>2</sup> per gram. In over two hundred runs,

the titanium powder produced by the Armstrong Process always has a packing fraction in the range of from about 4% to about 11% which also may also be expressed as tap density. Tap density is a well known characteristic and is determined by introducing the powder into a graduated test tube and tapping the tube until the powder is fully settled. Thereafter, the weight of the powder is measured and the packing fraction or percent of theoretical density is calculated.

Moreover, during the production of CP titanium by the Armstrong Process, a certain amount of sodium has always been retained even after extensive distillation, including vacuum distillation, and this retained sodium has been present on average of about 500-700 ppm, and has rarely been below about 400 ppm. From a commercial point of view, significant effort is and has been expended in order to reduce the sodium content of CP titanium made by the Armstrong Process.

Prior to the Armstrong Process, CP titanium powder and titanium alloy powder traditionally have been made by two methods, hydride-dehydride and spheridization, resulting in powders having very different morphologies than the powder made by the Armstrong method. Hydride-dehydride powders are angular and flake-like, while spheridized powders are spheres.

Fines made during the Hunter process are available and these also have very different morphology than CP titanium produced by the Armstrong Process. SEMs of CP powder made by the hydride-dehydride process and the spheridization process and Hunter fines are illustrated in FIGS. 1 to 3, respectively. The CP powder made by the Armstrong Process is not spherical nor is it angular and flake-like. Hunter fines have "large inclusions" which do not appear in the Armstrong powder, differentiating FIGS. 1-3 from Armstrong powder shown in FIGS. 4-9. Moreover, Hunter fines have large concentrations of chlorine while Armstrong CP powder has low concentrations of chlorine; chlorine is an undesirable contaminant.

6/4 powder is made by hydride-dehydride and spherization processes, but not by the Hunter process. A calcium reduction hydride-dehydride process used in Tula, Russia was identified by Moxson et al. in an article in The International Journal Of Powder Metallurgy, Vol. 34, No. 5, 1998. Moxson et al which also discloses SEMs of both CP and 6/4 in the Journal Of Metallurgy, May, 2000, both articles, the disclosures of which are incorporated by reference, taken together showing that 6/4 powder made by methods other than the Armstrong process result in powders that are very different from Armstrong 6/4 powder, both in size distribution and/or morphology and/or chemistry. In some cases, such as the calcium reduction process in Tula, Russia there are very significant differences in chemistry as well as the other differences previously mentioned. Both the hydride-dehydride and spheridization methods require Ti, Al and V to be mixed as liquids and thereafter formed into powder. Only the Armstrong Process produces alloy powder directly from gas mixtures of the alloy constituents.

Because 6/4 titanium is the most common titanium alloy used by the Department of Defense (DOD) as well as the aerospace industry and other significant industries, the production of 6/4 by the Armstrong Process is an important commercial goal.

#### SUMMARY OF THE INVENTION

Accordingly, a principal object of the present invention is to provide a titanium base alloy powder having lesser

amounts of aluminum and vanadium with unique morphological and chemical properties.

Another object of the present invention to provide a titanium base alloy powder having about 6 percent by weight aluminum and about 4 percent by weight vanadium within current ASTM specifications.

Yet another object of the invention is to make a 6/4 alloy as set forth in which sodium is present in significantly smaller amounts than is present in CP titanium powder made by the Armstrong Process.

Still another object of the present invention is to provide a titanium base alloy powder having about 6% by weight aluminum and about 4% by weight vanadium with an alkali or alkaline earth metal being present in an amount less than about 200 ppm and the alloy powder being neither spherical nor angular or flake shaped.

A further object of the present invention is to provide a titanium base alloy powder having about 6% by weight aluminum and about 4% by weight vanadium with an alkali or alkaline earth metal being present in an amount less than about 200 ppm and having a tap density or packing fraction in the range of from about 4% to about 11%.

Yet another object of the present invention is to provide a titanium base alloy powder having about 6% by weight aluminum and about 4% by weight vanadium with an alkali or an alkaline earth metal being present in an amount less than about 200 ppm made by the subsurface reduction of chloride vapor with molten alkali metal or molten alkaline earth metal.

A final object of the present invention is to provide an agglomerated titanium base alloy powder having about 6% by weight aluminum and about 4% by weight vanadium with an alkali or alkaline earth metal being present in an amount less than about 100 ppm substantially as seen in the SEMs of FIGS. 10-12.

The invention consists of certain novel features and a combination of parts hereinafter fully described, illustrated in the accompanying drawings, and particularly pointed out in the appended claims, it being understood that various changes in the details may be made without departing from the spirit, or sacrificing any of the advantages of the present invention.

#### BRIEF DESCRIPTION OF THE DRAWINGS

For the purpose of facilitating an understanding of the invention, there is illustrated in the accompanying drawings a preferred embodiment thereof, from an inspection of which, when considered in connection with the following description, the invention, its construction and operation, and many of its advantages should be readily understood and appreciated.

FIG. 1 is a SEM of CP powder made by the hydride-dehydride method;

FIG. 2 is a SEM of CP powder made by the spheridization method;

FIG. 3 is a SEM of CP powder from the Hunter Process;

FIGS. 4-6 are SEMs of Armstrong CP distilled, dried and passivated;

FIGS. 7-9 are SEMs of Armstrong CP distilled, dried, passivated and held at 750° C. for 48 hours; and

FIGS. 10-12 are SEMs of Armstrong 6/4 distilled, dried, passivated and held at 750° C. for 48 hours.

#### DETAILED DESCRIPTION OF THE INVENTION

As used herein, a "titanium base alloy" means any alloy having 50% or more by weight titanium. Although 6/4 is used as a specific example, other titanium base alloys are included

in this invention. As seen from the previous discussion, Armstrong CP titanium powder is different from spheridized titanium powder and from hydride-dehydride titanium powder in both morphology and packing fraction or tap density. There are also differences in certain of the chemical constituents. For instance, Armstrong CP titanium powder has sodium present in the 400-700 ppm range while spheridized and hydride-dehydride powder should have none or only trace amounts. Armstrong CP titanium has little chloride concentration, on the order of <50 ppm, while Hunter fines have much larger concentrations of chlorides, on the order of 0.12-0.15 wt. %.

The equipment used to produce the 6/4 alloy is substantially as disclosed in the aforementioned patents disclosing the Armstrong Process with the exception that instead of only having a titanium tetrachloride boiler 22 as illustrated in those patents, there is also a vanadium tetrachloride boiler and an aluminum trichloride boiler which are connected to the reaction chamber by suitable valves. The piping acts as a manifold so that the gases are completely mixed as they enter the reaction chamber and are introduced subsurface to the flow-

Na Flowrate=40 kg/min  
TiCl<sub>4</sub> Flowrate=2.6 kg/min

For this specific experiment, a 7/32" nozzle was used in the reactor to meter the mix of metal chloride vapors. A 0.040" nozzle was used to meter the AlCl<sub>3</sub> and a 0.035" nozzle was used to meter the VCl<sub>4</sub> into the TiCl<sub>4</sub> stream. The reactor was operated for approximately 250 seconds injecting approximately 11 kg of TiCl<sub>4</sub>. The salt and titanium alloy solids were captured on a wedge wire filter and free sodium metal was drained away. The product cake containing titanium alloy, sodium chloride and sodium was distilled at approximately 100 milli-torr at 550 to 575° C. vessel wall temperatures for 20 hours. Once all the sodium metal was removed via distillation, the trap was re-pressurized with argon gas and heated to 750° C. and held at temperature for 48 hours. The vessel containing the salt and titanium alloy cake was cooled and the cake was passivated with a 0.7 wt % oxygen/argon mixture. After passivation, the cake was washed with deionized water and subsequently dried in a vacuum oven at less than 100° C.

Table 2 below sets forth a chemical analysis of various runs for 6/4 alloy from an experimental loop running the Armstrong Process.

TABLE 2

| Ti 6/4 FROM EXPERIMENTAL LOOP |      |           |           |           |           |          |           |           |           |           |
|-------------------------------|------|-----------|-----------|-----------|-----------|----------|-----------|-----------|-----------|-----------|
| Run                           | Size | Oxygen    | Sodium    | Nitrogen  | Hydrogen  | Chloride | Vanadium  | Aluminum  | Carbon    | Iron      |
| N-269-                        | *    | 0.187     | 0.019     | 0.006     | 0.0029    | 0.001    | 5.58      | 5.58      | 0.019     | 0.014     |
| N-269-                        | +    | 0.113     | 0.0015    | 0.008     | 0.003     | 0.001    | 5.33      | 5.38      | 0.03      | 0.021     |
| N-269-                        | +    | 0.128     | 0.0006    | 0.005     | 0.0037    | 0.001    | 5.84      | 5.47      | 0.039     | 0.02      |
| N-271-                        | +    | 0.124     | 0.002     | 0.001     | 0.0066    | 0.0016   | 4.87      | 6.95      | 0.033     | 0.037     |
| N-276                         | +    | 0.111     | 0.0018    |           |           |          | 4.44      | 6.04      |           |           |
| N-276                         | +    | 0.121     | 0.0018    | 0.005     | 0.0043    | 0.0005   | 4.12      | 6.35      | 0.012     | 0.016     |
| N-276                         | +    | 0.131     | 0.0019    | 0.003     | 0.0057    | 0.0011   | 4.03      | 5.67      | 0.012     | 0.016     |
| N-276                         | +    | 0.169     | 0.0026    |           |           |          | 4.1       | 6.02      |           |           |
| N-276                         | +    | 0.128     | 0.0015    | 0.003     | 0.0042    | 0.0005   | 3.8       | 6.02      | 0.012     | 0.019     |
| N-277                         | +    | 0.155     | 0.0018    | 0.003     | 0.0053    | 0.0006   | 3.45      | 5.73      | 0.014     | 0.015     |
| N-277                         | +    | 0.135     | 0.0023    |           |           |          | 3.49      | 5.49      |           |           |
| N-276                         | *    | 0.121     | 0.0041    | 0.005     | 0.0052    | 0.0005   | 4.31      | 6.53      | 0.02      | 0.015     |
| N-276                         | *    | 0.134     | 0.0075    |           |           |          | 3.81      | 5.92      |           |           |
| N-276                         | *    | 0.175     | 0.014     | 0.012     | 0.0066    | 0.0005   | 3.96      | 6.01      |           |           |
| N-276                         | *    | 0.187     | 0.046     | 0.007     | 0.0081    | 0.0005   | 3.95      | 6.05      |           |           |
| N-277                         | *    | 0.141     | 0.0022    | 0.004     | 0.0038    | 0.0026   | 3.65      | 5.42      |           |           |
| mean                          |      | 0.14125   | 0.0069125 | 0.0051667 | 0.00495   | 0.00095  | 4.295625  | 5.914375  | 0.0212222 | 0.0192222 |
| stand dev                     |      | 0.0253811 | 0.0116064 | 0.0028868 | 0.0015952 | 0.000626 | 0.7343838 | 0.4335892 | 0.0102808 | 0.0071024 |

\* = BULK

+ = SMALL

ing liquid sodium. It was determined during production of the 6/4 alloy that aluminum trichloride is corrosive and required special materials not required for handling either titanium tetrachloride or vanadium tetrachloride. Therefore, Hastelloy C-276 was used for the aluminum trichloride boiler and the piping to the reaction chamber.

During most of the runs the steady state temperature of the reactor was maintained at about 400° C. by the use of sufficient excess sodium. Other operating conditions for the production of the alloy were as follows:

A device similar to that described in the incorporated Armstrong patents was used except that a VCl<sub>4</sub> boiler and AlCl<sub>3</sub> boiler were provided and both gases were fed into the line feeding TiCl<sub>4</sub> into the liquid Na. The boiler pressures and system parameters are listed hereafter.

#### Experimental Procedure:

TiCl<sub>4</sub> Boiler Pressure=500 kPa

VCl<sub>4</sub> Boiler Pressure=630 kPa

AlCl<sub>3</sub> Boiler Pressure=830 kPa

Inlet Na temperature=240° C.

Reactor Outlet Temperature=510 C

As seen from the above Table 2, the sodium levels for 6/4 are very low on the order of 69 ppm and for certain runs, sodium levels have been undetectable. This result was unexpected because over two hundred runs of CP titanium have been made using the Armstrong Process, and sodium has always been present in the range of from about 400-700 ppm. Therefore, the lack of sodium in the 6/4 alloy was not only unexpected but an important consideration since sodium may adversely affect the welds of CP titanium.

Other important aspects shown in Table 2 are the percentages of vanadium and aluminum in the 6/4 showing an average of about 5.91% aluminum and about 4.29% vanadium for all of the runs. The runs reported in Table 2 were made with an experimental loop and the valving and control systems for metering the appropriate amount of both vanadium and aluminum were rudimentary. Advanced valving systems have now been installed to control more closely the amount of vanadium and aluminum in the 6/4 produced from the Armstrong Process, although even with the rudimentary control system, the 6/4 alloy was within ASTM specifications. Also of significance is the low iron and chloride content of the 6/4 alloy.

An additional unexpected feature of the 6/4 alloy compared to the CP titanium is the surface area, as determined using BET Specific Surface Area analysis with krypton as the adsorbate. In general, the specific surface area of the 6/4 alloy is much larger than the CP titanium and this also was unexpected. Surface analysis of CP particles which were distilled overnight (about 8-12 hours) between 500-575° C. were 0.534 square meters/gram whereas 6/4 alloy measured 3.12 square meters/gram, indicating that the alloy is significantly smaller than the CP.

The SEMs show that the 6/4 powder is "frillier" than CP powder, see FIGS. 4-9 and 10-12. As reported by Moxson et al., *Innovations in Titanium Powder Processing* in the Journal of Metallurgy May 2000, it is clear that by-product fines from the Kroll or Hunter Processes contain large amounts of undesirable chlorine which is not present in the CP titanium powder made by the Armstrong Process (see Table 1). Moreover, the morphology of the Hunter and Kroll fines, as previously discussed, is different from the CP powder made by the Armstrong Process. Neither the Kroll nor the Hunter process has been adapted to produce 6/4 alloy. Alloy powders have been produced by melting prealloyed stock and thereafter using either gas atomization or a hydride-dehydride process (MHR). The Moxson et al. article discloses 6/4 powder made in Tula, Russia and as seen from FIG. 2 in that article, particularly FIGS. 2c and 2d the powders made by Tula Hydride Reduction process are significantly different than those made by the Armstrong Process. Moreover, referring to the Moxson et al. article in the 1998 issue of the International Journal of Powder Metallurgy, Vol. 4, No. 5, pages 45-47, it is seen that the chemical analysis for the pre-alloy 6/4 powder produced by the metal-hydride reduction (MHD) process contains exceptional amounts of calcium and also is not within ASTM specifications for aluminum.

Because the 6/4 alloy made by the Armstrong Process is made without the presence of either calcium or magnesium, these metals should be present, if at all, only in trace amounts and certainly much less than 100 ppm. Sodium which would be expected to be present in significant quantities based on the operation of the Armstrong Process to produce CP titanium in fact is present only at minimum quantities in the 6/4 alloy. Specifically, sodium in the 6/4 alloy made by the Armstrong Process is almost always present less than 200 ppm and generally less than 100 ppm. In some instances, 6/4 alloy has been produced using the Armstrong Process in which sodium is undetectable so that this is a great and unexpected advantage of the 6/4 alloy vis a vis CP titanium made by the Armstrong Process.

Both the Armstrong CP titanium and 6/4 alloy have tap densities or packing fractions in the range of from about 4% to 11%. This tap density or packing fraction is unique and inherent in the Armstrong Process and, while not advantageous particularly with respect to powder metallurgical processing, distinguishes the CP powder and the 6/4 powder made by the Armstrong Process from all other known powders.

As is well known in the art, solid objects can be made by forming 6/4 or CP titanium into a near net shapes and thereafter sintering, see the Moxson et al. article and can also be formed by hot isostatic pressing, laser deposition, metal injecting molding, direct powder rolling or various other well known techniques. Therefore, the titanium alloy powder made by the Armstrong method may be formed into a sintered product or may be formed into a solid object by well known methods in the art and the subject invention is intended to cover all such products made from the powder of the subject invention.

While the invention has been particularly shown and described with reference to a preferred embodiment hereof, it will be understood by those skilled in the art that several changes in form and detail may be made without departing from the spirit and scope of the invention which includes titanium base alloys having lesser amounts of aluminum and vanadium and is specifically not limited to the specific alloys disclosed.

We claim:

- 10 1. A titanium base alloy powder comprising:  
pre-alloy particles, a majority of the pre-alloy particles  
having a composition of at least 50% by weight of titanium,  
5.38% or more by weight of aluminum, 3.45% or  
more by weight of vanadium, and less than about 200  
ppm alkali or alkaline earth metal, wherein the total  
amount of aluminum and vanadium is less than about  
20% by weight, and wherein  
the titanium base alloy powder has a tap density in a range  
of from about 4% to about 11% and a Brunauer, Emmett,  
and Teller (BET) specific surface area of at least about 3  
square meters per gram, and meets ASTM B265 grade 5  
chemical specifications.
- 15 2. The alloy powder of claim 1, wherein said alloy powder  
comprises agglomerates having an average mean diameter as  
measured by sieve analysis greater than about 50 microns.
- 20 3. The alloy powder of claim 1, wherein sodium and mag-  
nesium and calcium are present in an amount of less than  
about 100 ppm.
- 25 4. The alloy powder of claim 1 formed into a sintered  
product.
- 30 5. A solid object made from the alloy powder of claim 1.
- 35 6. The alloy powder of claim 1 wherein the aluminum is in  
a range of 5.38% to 6.95% by weight and the vanadium is in  
a range of 3.45% to 4.87% by weight.
- 40 7. The alloy powder of claim 1 wherein the majority of  
pre-alloy particles are neither spherical nor angular and flake  
shaped.
- 45 8. A titanium base alloy powder comprising:  
pre-alloy particles, a majority of the pre-alloy particles  
having 50% or more by weight of titanium, about 5.38%  
to 6.95% by weight of aluminum and about 3% to about  
5% by weight of vanadium, and wherein  
the titanium base alloy powder has an alkali or alkaline  
earth metal content of less than about 200 ppm, a tap  
density in a range of from about 4% to about 11%, and a  
Brunauer, Emmett, and Teller (BET) specific surface  
area of at least about 3 square meters per gram, and  
meets ASTM B265 grade 5 chemical specifications.
- 50 9. The alloy of claim 8, wherein said alloy powder com-  
prises agglomerates having an average mean diameter as  
measured by sieve analysis greater than about 50 microns.
- 55 10. The alloy powder of claim 8, wherein sodium and mag-  
nesium and calcium are present in an amount of less than  
about 100 ppm.
- 60 11. The alloy powder of claim 8 agglomerated as seen in  
FIGS. 10-12.
- 65 12. The alloy powder of claim 8 formed into a sintered  
product.
13. A solid object made from the alloy powder of claim 8.
14. The alloy powder of claim 8 wherein the aluminum in  
the majority of pre-alloy particles is in a range of 5.5% to  
6.75% by weight and the vanadium is in a range of 3.45% to  
4.87% by weight.
15. The alloy powder of claim 8 wherein the pre-alloy  
particles are neither spherical nor angular and flake shaped.
- 65 16. A titanium base alloy powder comprising pre-alloy  
particles, each pre-alloy particle having:

50% or more by weight of titanium, about 5.38% or more by weight of aluminum and about 3.45% or more by weight of vanadium, wherein the total amount of aluminum and vanadium is less than about 20% by weight, and an alkali or alkaline earth metal present in the alloy in an amount less than about 200 ppm, and wherein the titanium base alloy powder has a tap density in a range of from about 4% to about 11% and a Brunauer, Emmett, and Teller (BET) specific surface area of at least about 3 square meters per gram, and meets ASTM B265 grade 5 chemical specifications.

17. The alloy powder of claim 16, wherein sodium and calcium and magnesium are present in the pre-alloy particles in an amount of less than about 100 ppm.

18. The alloy powder of claim 16 agglomerated as seen in FIGS. 10-12.

19. The alloy powder of claim 16 formed into a sintered product.

20. A solid object made from the alloy powder of claim 16.

21. The alloy powder of claim 16 wherein the aluminum in each pre-alloy particle is in a range of 5.38% to 6.95% by weight and the vanadium is in a range of 3.45% to 4.87% by weight.

22. The alloy powder of claim 16 wherein the pre-alloy particles are neither spherical nor angular and flake shaped.

23. A titanium base alloy powder having:

pre-alloy particles, a majority of the pre-alloy particles having a composition of 50% or more by weight of titanium, 5.38% to 6.95% by weight of aluminum and 3% to 5% by weight of vanadium, and an alkali or an alkaline earth metal content of less than about 200 ppm, the pre-alloy particles made by the subsurface reduction of a chloride vapor with a molten alkali metal or a molten alkaline earth metal, and wherein the titanium base alloy powder has a tap density in a range of from about 4% to about 11%, has a Brunauer, Emmett, and Teller (BET) specific surface area of at least about 3 square meters per gram, and meets ASTM B265 grade 5 chemical specifications.

24. The alloy powder of claim 23, wherein sodium and calcium and magnesium are present in the pre-alloy particles in an amount of less than about 100 ppm.

25. The alloy powder of claim 23, wherein the molten alkali metal is flowing liquid sodium and the chloride vapor is introduced at greater than sonic velocity into the flowing liquid sodium.

26. The alloy powder of claim 23 agglomerated as seen in FIGS. 10-12.

27. The alloy powder of claim 23 formed into a sintered product.

28. A solid object made from the alloy powder of claim 23.

29. The alloy powder of claim 23 wherein the aluminum in the majority of pre-alloy particles is in a range of 5.5% to 6.75% by weight and the vanadium is in a range of 3.45% to 4.87% by weight.

30. The alloy powder of claim 23 wherein the pre-alloy particles are neither spherical nor angular and flake shaped.

31. A titanium base alloy powder comprising:

pre-alloy particles, each pre-alloy particle having 50% or more by weight of titanium, about 5.38% to 6.95% by weight of aluminum and about 3% to about 5% by weight of vanadium, and an alkali or alkaline earth metal present in an amount less than about 100 ppm, the pre-alloy particles agglomerated substantially as seen in FIGS. 10-12, and wherein the titanium base alloy powder has a tap density in a range of from about 4% to about 11%, has a Brunauer, Emmett, and Teller (BET) specific surface area of at least about 3 square meters per gram, and meets ASTM B265 grade 5 chemical specifications.

32. The alloy powder of claim 31 formed into a sintered product.

33. A solid object made from the alloy powder of claim 31.

34. The alloy powder of claim 31 wherein the aluminum in each pre-alloy particle is in a range of 5.5% to 6.75% by weight and the vanadium is in a range of 3.45% to 4.87% by weight.

35. The alloy powder of claim 31 wherein the pre-alloy particles are neither spherical nor angular and flake shaped.

\* \* \* \* \*